# EUROPEAN PATENT SPECIFICATION

(11) **EP 1 382 744 B1**
(45) Date of publication and mention of the grant of the patent: **03.03.2004**
(21) Application number: 02077577.1
(22) Date of filing: 28.06.2002
(51) Int. Cl.: D21H 27/00, B65D 57/00, B41C 1/10, G03F 7/00

(54) **Interleaf paper for printing plates**
Zwischenblattpapier für Druckplatten
Feuille de papier intercalaire pour plaques d'impression

(43) Date of publication of application: 21.01.2004
(73) Proprietor: Fuji Photo Film B.V., 5047 TK Tilburg (NL)
(72) Inventor: Imaizumi, Mitsuhiro, 5045 JG Tilburg (NL); Mangré, Randhiersing, 5165 EH Waspik (NL); Sekiya, Toshiyuki, 5045 JW Tilburg (NL)
(74) Representative: Prins, Adrianus Willem

(56) References cited:
- EP-A- 1 190 850
- US-A1- 2002 042 021
- DATABASE WPI Section Ch, Week 200240 Derwent Publications Ltd., London, GB; Class F09, AN 2002-367457 XP002220048 & JP 2002 054090 A (YUKO SHIKO KK), 19 February 2002 (2002-02-19)
- PATENT ABSTRACTS OF JAPAN vol. 2000, no. 25, 12 April 2001 (2001-04-12) & JP 2001 233385 A (FUJI PHOTO FILM CO LTD), 28 August 2001 (2001-08-28)

## Description

### Field of the invention

This invention relates to a photosensitive lithographic printing plate, particularly to the interleaf paper for the printing plate. When photosensitive lithographic printing plate is manufactured, a thin paper cover is applied on top of the photosensitive layer with a static electricity charge to prevent scratches and keep the photosensitive layer stable from environmental change. This paper cover is called interleaf paper which this invention relates to.

### Background of the invention

Recently in photosensitive lithographic printing plate market, the usage of thermal type computer to plate system is increasing. Advantage of the system is as follows. The plate can be exposed in infra-red wavelength directly from image data without using film. Similar or same processor and chemistry as the conventional system can be used. No change of the lighting conditions at the working room to handle the printing plate is necessary as the one used within the current conventional system, or even can be changed back to normal white light environment. Further more, all major plate setter vendors who have developed the exposure machines for this thermal type computer to plate system, have also developed autoloaders to load the printing plates automatically to their infra-red wavelength exposure system. This reduced the necessary manpower for handling printing plates. These advantages contribute in a positive way to increase the thermal type computer to plate system.

When the autoloaders load the printing plate into its exposure unit, it separates the printing plate and the interleaf paper. Some loaders which need manual operation to separate the interleaf paper from the printing plate are called semi-automatic loaders. In all autoloaders, first a bundle of printing plates is set, wherein in most cases the photosensitive layer side of the printing plate (= top side of the printing plate) is placed downwards to the ground. In this type of autoloader, the printing plate is picked up from the back side of the printing plate where there is no photosensitive layer. When the printing plate is picked up, it is important that the interleaf paper on the top side of the printing plate (facing downward) separates well from the picked up printing plate. After the printing plate is loaded, picking up of the remaining interleaf paper from the back side of the next printing plate is not so critical since there is no electrostatic charge applied in between the interleaf paper and the backside of the next printing plate.

In other types of autoloaders, a bundle of printing plates is set first with the photosensitive layer of the printing plate (= top side of the printing plate) is placed upwards into the sky. In this type of autoloader, the printing plate is picked up from the top side of the printing plate. When the printing plate is picked up, it is important that the interleaf paper on the backside (facing downward) of the printing plate separates well from the printing plate. This separation is not as critical as the former case between the top side of the printing plate and the interleaf paper because at the production facility the topside of the printing plate is adhered together with the interleaf paper by electro statically charging means and not to the back side of the next printing plate. After the printing plate is loaded, the interleaf paper is picked up from the topside of the printing plate and the next printing plate will be loaded again etc.

However in the case when the back side of the printing plate is picked up by the autoloader, another problem is experienced sometimes as the interleaf paper sticks to the topside of the printing plate. This happens to a smaller extent also when the top side of the printing plate is picked up, but the picking up of the printing plate from the backside is more critical. When this interleaf paper does not fall down, the interleaf paper will be loaded together with the printing plate into the exposure unit which causes an incorrect exposure or a machine stop. As worst case a printing plate underneath can also be picked up at the same time, which causes a double loading. These machine failures consume extra manpower to recover the condition, and much operational time for solving this problem is also lost.

Another problem can happen when the autoloader is picking up the interleaf paper by suction cups. Problems are experienced when the suction cups pick up the interleaf paper together with the printing plate underneath. This causes a jam in the waste paper container, which requires again extra manpower and waste of operational time.

Further more, another problem can happen when the interleaf paper is picked up by the suction cups at the autoloader, when the autoloader interprets wrongly that the paper is not picked up. This happens more when some of the suction cups are not in use due to the size of the printing plate or by any malfunctioning of the suction cups. In such a case, the vacuum alarm setting of the suction cups system has to be tuned, again with extra manpower consumption and operational time loss as well as high risk of not picking up of the interleaf paper correctly.

Another problem in the market is that when the interleaf paper is sent to the waste paper container of the autoloader, sometimes less paper can be put in since the alarm for the waste container is activated. This will not be recovered until the waste interleaf paper is removed from the waste paper container. This also causes extra manpower consumption and operational time loss.

Even further, there is a problem that at certain sizes of printing plates, the distance between the active suction cups at the edge and the edge of the plate is too big and the paper starts to bend down. When this happens in front of the guide roller, the paper is no longer guided through the guide roller but gives a paper jam at this roller. Again, this causes extra manpower consumption and operational time loss.

### Summary of the invention / itemized

With the information above, an object of the present invention is to provide selection criteria of the interleaf paper suitable for these autoloaders. Main aspect is to prevent any stop of the autoloader such that no loss of manpower and operational time happen.

First aspect is to prevent sticking of the interleaf paper to the picked up printing plate. According to the present invention this can be solved by keeping the paper surface rough enough such that the air can intervene between the interleaf paper and the printing plate. When enough air can intervene, the interleaf paper can easily be separated from the printing plate.

Second aspect is to prevent picking up the printing plate when the interleaf paper is picked up by the suction cups. According to the present invention this problem can be solved by keeping the air permeability high enough such that less air goes through the paper. When the air does not go through, no vacuum will be formed between the interleaf paper and the printing plate.

Third aspect is to prevent that the waste interleaf paper will fill the waste paper container very quickly. According to the present invention this problem can be solved by keeping the bending stiffness of the paper low enough such

US-A-2002/042021 discloses an overleaf paper for separating photosensitive printing plates having a Bekk smoothness at the side facing the photosensitive layer of less than 30 seconds [0026], a stiffness of 100 g or higher and a stiffness per unit thickness of 2.0 g/cm or higher [0028]. that the waste paper can be wrinkled easily into a smaller volume, which allows more paper to be put into the waste paper container.

Fourth aspect is to prevent that the corner of the interleaf paper bends in front of the paper guide roller. According to the present invention this problem can be solved by keeping the bending stiffness of the paper high enough such that corner bending does not occur.

Fifth aspect is to use paper without synthetic polymer to allow paper recycling.

For a better understanding of the present invention examples of an interleaf paper, stack of printing plates with such interleaf papers in between and a method for loading such printing plates are described by way of example only. In general in a method according to the present invention interleaf paper is chosen such that it separates easily from a printing plate. Preferably they separate under gravity within approximately a second or less after picking up.

### Examples

### Preparation of photosensitive printing plate

In the examples as photosensitive printing plate the thermal positive printing plate LH-PIE manufactured by Fuji Photo Film BV was applied. Here below examples are shown of interleaf papers according to the prior art in comparison to interleaf papers according to the present invention. The interleaf papers according to the present invention include the papers referred to as samples. Examples of possible substrate treatments are e.g. shown in JP10282645, JP10301262. Suitable coating materials are shown in JP2000241962, JP2000241961, JP2000112136, JP2000112132, JP2000112135, EP1182033, EP1182032, EP1170123, EP1096315, EP1155820, EP1129845.

For the interleaf paper various commercial papers of less than 100g/m2 gram mage (determined by ISO 536 standard procedure) are used. The properties of the papers used are shown in Table 1.

The thickness of the paper is measured by a micrometer according to ISO 534. Bekk smoothness is measured by a smoothness meter according to the ISO 8791-1 standard procedure. The Bekk air permeability of the paper is measured by an air permeability meter according to ISO 5636-1 standard procedure. Bending stiffness of the paper is measured by a stiffness meter according to the ISO 5628 standard procedure. Tensile strength is measured by tensile strength tester according to ISO 1924-2.

The term "machine" direction is referring to an orientation in the direction of a paper web which is adhered in the manufacturing process of the printing plate; the term "cross" direction is referring to an orientation in the plane of the paper web and perpendicular to the "machine" direction. The limits given in the description should be assessed within the gist of the invention.

**Table 1.**

| Properties of papers used for interleaf | | | | | | | |
|---|---|---|---|---|---|---|---|
| | Syntheti Polyme | Pape Appearan | Thicknes micron | Smoothne Bekk | Air permeability Bekk | Bending Stiffness | |
| | | | | | | MD | CD |
| Sample | Not | Both sides | 60 | 20 | 85 | 28 | 11 |
| Sample | Not | Roth sides | 55 | 25 | 50 | 36 | 11 |
| Refernce | Not | Both sides | 47 | 25 | 30 | 7 | 4 |
| Refernce | Not | Both sides | 72 | 30 | 3 | 48 | 20 |
| Refernce | Not | Both sides | 47 | 35 | 30 | 10 | 3 |
| Refernce | Not | One side | 62 | 50 | 10 | 21 | 7 |
| Refernce | Not | One side | 45 | 65 | 2 | 14 | 6 |
| Refernce | Not | One side | 79 | 100 | 2 | 30 | 16 |
| Refernce | Not | One side | 57 | 150 | 1 | 11 | 3 |
| Refernce | Not | One side | 54 | 290 | 14 | 11 | 3 |
| Refernce | Not | One side | 44 | 300 | 15 | 7 | < 1 |
| Refernce | Use | One side | 38 | 600 | 2000 | < 1 | < 1 |
| MD = machine direction CD = cross | | | | | | | |

### Sticking Test

For each interleaf paper type bundles of 30 printing plate sheets were cut into 400mm x 500mm. 3 bundles of each interleaf paper type was set on a table with the photosensitive layer facing downwards to the ground. The printing plate was picked up from the back side of the printing plate by an arm with 4 suction cups. When the plate is picked up, sometime later the interleaf paper underneath the picked up plate falls down and separates from the plate. The necessary time for the interleaf paper to fall was measured in seconds. After removing the interleaf paper manually, the next plate was picked up by the same procedure. In worst cases, a plate underneath the interleaf was also picked up. After 90 sheets are picked up, another 3 bundles were set on a table with the photosensitive layer facing upwards to the sky. The same picking up test was done again. The percentage of sheets consuming more than 2 seconds to separate the interleaf paper from the plate was calculated and defined as interleaf sticking paper percentage. The data is shown in Table 2.

**Table 2.**

| Result of sticking test | | | | | |
|---|---|---|---|---|---|
| | Synthetic Polymer | Paper Appearance | Thickness microns | Smoothness Bekk sec | Sticking % |
| Sample 1 | Not used | Both sides rough | 60 | 20 sec | 0 |
| Sample 2 | Not used | Both sides rough | 55 | 25 sec | 0 |
| Refernce 1 | Not used | Both sides rough | 47 | 25 sec | 0 |
| Refernce 2 | Not used | Both sides rough | 72 | 30 sec | 0 |
| Refernce 3 | Not used | Both sides rough | 47 | 35 sec | 0 |
| Refernce 4 | Not used | One side smooth | 62 | 50 sec | 10 |
| Refernce 5 | Not used | One side smooth | 45 | 65 sec | 30 |
| Refernce 6 | Not used | One side smooth | 79 | 100 sec | 30 |
| Refernce 7 | Not used | One side smooth | 57 | 150 sec | 60 |
| Refernce 10 | Not used | One side smooth | 54 | 290 sec | 100 |
| Refernce 8 | Not used | One side smooth | 44 | 300 sec | 100 |
| Refernce 9 | Used | One side coated | 38 | 600 sec | 100 |

As shown in Table 2, the smoothness measurement must be lower than approximately 40 Bekk seconds to achieve a sticking percentage of 0%. Due to a low Bekk sec Smoothness it is surprisingly shown that air can relatively easily enter between the plate surface and the interleaf paper, thus preventing under pressure in between. The result shows clearly how important it is for the air to leak in between the picked up printing plate and the interleaf paper underneath to let paper fall easily. By providing sufficiently low smoothness air will be allowed to escape between the PS plate and the interleaf paper.

### Plate pick up through paper test

For each interleaf paper type bundles of 30 printing plate sheets were cut into 400mm x 500mm. 3 bundles of printing plate with each interleaf paper type respectively was set on a table with the photosensitive layer facing downwards to the ground. After taking of the top printing plate, interleaf paper was picked up from the back side of the printing plate by an arm with 4 suction cups. When the interleaf paper was picked up, sometimes later the printing plate underneath the picked up interleaf paper falls down and separates from the interleaf paper. The necessary time for the plate to fall was measured in seconds. After removing the printing plate manually, the next interleaf paper was picked up by the same procedure. After 90 sheets of interleaf paper were picked up, another 3 bundles were set on a table with the photosensitive layer facing upwards to the sky. Same picking up test was done again. The percentages of sheets consuming more than 1, 2 or 3 seconds to separate the interleaf paper from the printing plate were calculated and defined as plate pickup percentage through paper. The result is shown in Table 3. As clearly shown in Table 3, the Bekk air permeability must be higher than approximately 40 seconds to prevent plate pickup through interleaf paper, even in the one sec. test.

**Table 3.**

| Results of plate pickup through paper test and vacuum alarm test | | | | | | | | |
|---|---|---|---|---|---|---|---|---|
| | Synthetic Polymer | Paper Appearance | Thickness microns | Air permeability Bekk sec | Plate pickup through paper (%) | | | Vacuum alarm (% |
| | | | | | > 1 sec | > 2 sec | > 3 sec | |
| Sample 1 | Not used | Both sides rough | 60 | 85 sec | 0 | 0 | 0 | 0 |
| Sample 2 | Not used | Both sides rough | 55 | 50 sec | 0 | 0 | 0 | 0 |
| Refernce 9 | Used | One side coated | 38 | 2000 sec | 0 | 0 | 0 | 0 |
| Refernce 1 | Not used | Both sides rough | 47 | 30 sec | 10 | 5 | 0 | 0 |
| Refernce 3 | Not used | Both sides rough | 47 | 30 sec | 10 | 5 | 0 | 0 |
| Refernce 8 | Not used | One side smooth | 44 | 15 sec | 10 | 5 | 0 | 0 |
| Refernce 10 | Not used | One side smooth | 54 | 14 sec | 10 | 5 | 0 | 0 |
| Refernce 4 | Not used | One side smooth | 62 | 10 sec | 10 | 5 | 0 | 0 |
| Refernce 2 | Not used | Both sides rough | 72 | 3 sec | 20 | 5 | 0 | 0 |
| Refernce 5 | Not used | One side smooth | 45 | 2 sec | 40 | 30 | 5 | 5 |
| Refernce 6 | Not used | One side smooth | 79 | 2 sec | 40 | 30 | 5 | 5 |
| Refernce 7 | Not used | One side smooth | 57 | 1 sec | 90 | 50 | 30 | 30 |

### Vacuum alarm test

For each interleaf paper type bundles of 30 printing plate sheets were cut into 1030mm x 790mm. 3 bundles of printing plates, with each interleaf paper type respectively were set into a Fujifilm SAL-9000 autoloader. In a cassette, plates were set with the photosensitive layer facing downwards to the ground. After taking out the top printing plate, interleaf paper was picked up from the back side of the printing plate by the autoloader arm. A pressure gauge of the suction cup vacuum system was checked, and the percentage that the vacuum level of holding the interleaf paper goes below 60% of that when the printing plate was held up was calculated as vacuum alarm. The lowest moment was when the interleaf paper was picked up and was separated from the printing plate underneath. The alarm is normally set to about 50%. It is clear to see from Table 3 that especially very low Bekk air permeability results in a vacuum alarm.

### Stiffness related tests

For each interleaf paper type, bundles of 30 printing plate sheets were cut into 1030mm x 790mm. 3 bundles of printing plates with each interleaf paper type respectively were set into a Fujifilm SAL-9000 autoloader. In a cassette, plates were set with the photosensitive layer facing downwards to the ground. Loading tests were done for these 90 sheets of each type of interleaf paper, and the waste paper container after the machine was observed closely. The same test was done with a CreoScitex Lotem 800 autoloader and a CreoScitex Trendsetter 5880 AL without compressing unit. The filling efficiency of the waste paper container was tested to see if 30 sheets of interleaf paper can be sent easily into the waste container or not. As shown in Table 4, the bending stiffness of the interleaf paper in the machine direction must be lower than approximately 42mN to have good efficiency usage of the waste paper container.
To test the corner bend behaviour for each interleaf paper type, bundles of 30 printing plate sheets were cut into 400mm machine direction x 500mm cross direction. 3 bundles with each interleaf paper type respectively were set on a table with the photosensitive layer facing downwards to the ground. After taking of the top printing plate, interleaf paper was picked up from the back side of the printing plate by an arm with 4 suction cups. Suction cups were positioned 150 mm away from the 400mm length edge. When the interleaf paper was picked up at the height of 100mm, corner bending of the interleaf paper was observed visually for various reference papers. As shown in Table 4, the bending stiffness of the interleaf paper in the cross direction must be higher than approximately 8mN in order to have good corner bending.

The thickness of the interleaf sheets is preferably less than approximately 70 microns since then a desired number of plates can be attached and packed in a box commonly used. The sheets may be thicker than 45 micron in order to be handled more easily.

**Table 4.**

| Results of waste bin efficiency test and corner bending test | | | | | | | |
|---|---|---|---|---|---|---|---|
| | Synthetic Polymer | Paper Appearance | Thickness microns | Bending Stiffness (mN) | | Waste bin efficiency | Corner bending |
| | | | | MD | CD | | |
| Sample 1 | Not used | Both sides rough | 60 | 28 | 11 | good | good |
| Sample 2 | Not used | Both sides rough | 55 | 36 | 11 | good | good |
| Refernce 2 | Not used | Both sides rough | 72 | 48 | 20 | bad | good |
| Refernce 6 | Not used | One side smooth | 79 | 30 | 16 | good | good |
| Refernce 4 | Not used | One side smooth | 62 | 21 | 7 | good | not good |
| Refernce 5 | Not used | One side smooth | 45 | 14 | 6 | good | not good |
| Refernce 7 | Not used | One side smooth | 57 | 11 | 3 | good | not good |
| Refernce 10 | Not used | One side smooth | 54 | 11 | 3 | good | not good |
| Refernce 3 | Not used | Both sides rough | 47 | 10 | 3 | good | bad |
| Refernce 1 | Not used | Both sides rough | 47 | 7 | 4 | good | not good |
| Refernce 8 | Not used | One side smooth | 44 | 7 | < 1 | good | bad |
| Refernce 9 | Used | One side coated | 38 | < 1 | < 1 | good | bad |
| MD = machine direction CD = cross direction | | | | | | | |

The present invention is by no means limited to the examples shown. Many variations are possible within the scope of the invention as defined by the claims. Any combination of material properties according to the present invention especially as discussed in the examples is considered to be included in this description as falling within said scope.

## Claims

1. An interleaf paper for photosensitive printing plate wherein the Bekk smoothness of the interleaf paper at the side facing the photosensitive layer is less than 40 seconds, and Bekk air permeability is more than 40 seconds.

2. An interleaf paper preferably according to claim 1 for photosensitive printing plate which is sensitive to infra-red wavelength exposure.

3. An interleaf paper according to claim 1 or 2 wherein bending stiffness of the interleaf paper at the cross direction of the paper is higher than 8mN and at the machine direction of the paper lower than 42 mN.

4. An interleaf paper according to anyone of claims 1 - 3 wherein the thickness of the paper is less than approximately 70 microns.

5. An interleaf paper according to anyone of claims 1 - 4 wherein the density of the paper is more than approximately 0.5 g/cm3.

6. An interleaf paper according to anyone of claims 1 - 5 wherein the tensile strength of the paper is higher than 1.5kN/m.

7. An interleaf paper according to anyone of claims 1 - 6 wherein the paper can be recycled, and is preferably made without plastic material, especially without a synthetic polymer.

8. Stack of printing plates, comprising interleaf papers according to anyone of claims 1- 7 in between said printing plates.

9. Stack of printing plates according to claim 8, wherein the Bekk smoothness of the or each into leaf paper is less than 40 seconds and facing the printing plate opposite the side facing up while the Bekk air permeability is more than 40 seconds.

10. Stack of printing plates according to claim 8 or 9, wherein the Bekk smoothness of the or reach into leaf paper is less than 40 seconds and facing the printing plate on the side facing up, while the Bekk air permeability is more than 40 seconds.

11. Method for loading printing plates from a stack according to anyone of claims 8 - 10, wherein the interleaf paper is chosen such that air is allowed to enter in between the paper and an adjacent printing plate such that the interleaf paper and the printing plate, when picked up, separate within less than 1 second after picking up.

## Patentansprüche

1. Durchschussbogenpapier für eine fotoempfindliche Druckplatte, wobei die Bekk-Glätte des Durchschussbogenpapiers an der Seite, die der fotoempfindlichen Schicht zugewandt ist, weniger als 40 Sekunden beträgt und die Bekk-Luftdurchlässigkeit mehr als 40 Sekunden beträgt.

2. Durchschussbogenpapier vorzugsweise nach Anspruch 1 für eine fotoempfindliche Druckplatte, das empfindlich für Belichtung mit Infrarotwellenlänge ist.

3. Durchschussbogenpapier nach Anspruch 1 oder 2, wobei die Biegesteifigkeit des Durchschussbogenpapiers in der Querrichtung des Papiers mehr als 8 mN und in der Maschinenrichtung des Papiers weniger als 42 mN beträgt.

4. Durchschussbogenpapier nach einem der Ansprüche 1-3, wobei die Dicke des Papiers weniger als etwa 70 µm beträgt.

5. Durchschussbogenpapier nach einem der Ansprüche 1-4, wobei die Dichte des Papiers mehr als etwa 0,5 g/cm³ beträgt.

6. Durchschussbogenpapier nach einem der Ansprüche 1-5, wobei die Zugfestigkeit des Papiers mehr als 1,5 kN/m beträgt.

7. Durchschussbogenpapier nach einem der Ansprüche 1-6, wobei das Papier recycelt werden kann und vorzugsweise ohne Kunststoffmaterial, insbesondere ohne synthetisches Polymer, hergestellt wird.

8. Stapel von Druckplatten, der Durchschussbogenpapiere nach einem der Ansprüche 1-7 zwischen den Druckplatten umfasst.

9. Stapel von Druckplatten nach Anspruch 8, wobei die Bekk-Glätte des oder jedes Durchschussbogenpapiers weniger als 40 Sekunden der Druckplatte zugewandt gegenüber der nach oben gewandten Seite beträgt, während die Bekk-Luftdurchlässigkeit mehr als 40 Sekunden beträgt.

10. Stapel von Druckplatten nach Anspruch 8 oder 9, wobei die Bekk-Glätte des oder jedes Durchschussbogenpapiers weniger als 40 Sekunden der Druckplatte zugewandt an der nach oben gewandten Seite beträgt, während die Bekk-Luftdurchlässigkeit mehr als 40 Sekunden beträgt.

11. Verfahren zum Einlegen von Druckplatten von einem Stapel nach einem der Ansprüche 8-10, wobei das Durchschussbogenpapier so ausgewählt wird, dass Luft zwischen das Papier und eine angrenzende Druckplatte eintreten kann, so dass sich das Durchschussbogenpapier und die Druckplatte, wenn sie angehoben wird, innerhalb von weniger als einer Sekunde nach dem Anheben trennen.

## Revendications

1. Feuille de papier intercalaire pour une plaque d'impression photosensible, dans laquelle le lissé Bekk de la feuille intercalaire sur le côté en face de la couche photosensible est inférieur à 40 secondes et la perméabilité à l'air Bekk est supérieure à 40 secondes.

2. Feuille de papier intercalaire de préférence selon la revendication 1 pour une plaque d'impression photosensible qui est sensible à une exposition à une longueur d'onde infrarouge.

3. Feuille de papier intercalaire selon la revendication 1 ou la revendication 2, dans laquelle la rigidité de pliage de la feuille de papier intercalaire suivant la direction transversale du papier est supérieure à 8 mN et suivant la direction machine du papier, inférieure à 42 mN.

4. Feuille de papier intercalaire selon l'une quelconque des revendications 1 à 3, dans laquelle l'épaisseur du papier est inférieure à environ 70 microns.

5. Feuille de papier intercalaire selon l'une quelconque des revendications 1 à 4, dans laquelle la densité du papier est supérieure à environ 0,5 g/cm³.

6. Feuille de papier intercalaire selon l'une quelconque des revendications 1 à 5, dans laquelle la résistance à la rupture par traction du papier est supérieure à 1,5 kN/m.

7. Feuille de papier intercalaire selon l'une quelconque des revendications 1 à 6, dans laquelle le papier peut être recyclé et est de préférence réalisé sans matière plastique, surtout sans polymère synthétique.

8. Pile de plaques d'impression, comprenant des feuilles de papier intercalaires, selon l'une quelconque des revendications 1 à 7, entre lesdites plaques d'impression.

9. Pile de plaques d'impression selon la revendication 8, dans laquelle le lissé Bekk de la ou de chacune des feuilles de papier est inférieur à 40 secondes et en face de la plaque d'impression opposée au côté se présentant de face vers le haut tandis que la perméabilité à l'air de Bekk est supérieure à 40 secondes.

10. Pile de plaques d'impression selon la revendication 8 ou la revendication 9, dans laquelle le lissé Bekk de la ou de chacune des feuilles de papier est inférieur à 40 secondes et en face de la plaque d'impression sur le côté se présentant de face vers le haut tandis que la perméabilité à l'air de Bekk est supérieure à 40 secondes.

11. Procédé pour charger des plaques d'impression à partir d'une pile selon l'une quelconque des revendications 8 à 10, dans lequel la feuille de papier intercalaire est sélectionnée de sorte que l'air puisse pénétrer entre le papier et une plaque d'impression adjacente, de sorte que la feuille de papier intercalaire et la plaque d'impression, lorsque celle-ci est saisie, se sépare en moins d'une seconde après la saisie.
